

E. J. TURNER & B. H. HOWARD.  
ADJUSTABLE FEEDER FOR STANDARD INGOT MOLDS.  
APPLICATION FILED APR. 30, 1915.

1,149,228.

Patented Aug. 10, 1915.

Fig. 1.



Fig. 3.



Fig. 2.



Fig. 6.



Fig. 7.



Witnesses

J. D. Ecker  
S. V. Goodall

Inventors

Ernest J. Turner  
Bloomfield H. Howard

# UNITED STATES PATENT OFFICE.

ERNEST J. TURNER, OF PITTSBURGH, AND BLOOMFIELD H. HOWARD, OF ASPINWALL, PENNSYLVANIA.

## ADJUSTABLE FEEDER FOR STANDARD INGOT-MOLDS.

1,149,228.

Specification of Letters Patent.

Patented Aug. 10, 1915.

Application filed April 30, 1915. Serial No. 24,913.

To all whom it may concern:

Be it known that we, ERNEST J. TURNER and BLOOMFIELD H. HOWARD, citizens of the United States, and residents, respectively, 5 of Pittsburgh, in the county of Allegheny and State of Pennsylvania, and of Aspinwall, in the county of Allegheny and State of Pennsylvania, have invented certain new and useful Improvements in Adjustable Feeders for Standard Ingot-Molds, of which the following is a specification.

Our invention relates to the manufacture of iron or steel ingots and has for its object to prevent, or reduce to a minimum the 15 formation of cavities, holes or seams known as "piping" in the upper portion of the ingot.

A further object of the invention is to provide an adjustable feeder made of furnace sand, fire clay or other refractory material that may be used with any standard 20 ingot mold.

A still further object of our invention is to provide a novel means for adjusting the 25 feeder so as to extend down into the mold any desired distance.

Other objects and advantages of our invention will appear in the course of the description.

30 A practical embodiment of our invention is represented in the accompanying drawings forming a part of this specification and in which like letters are employed to designate like parts throughout the several views.

35 Figure 1 is a sectional plan view of the preferred form of the feeder; Fig. 2 is a side view showing it applied to a mold; Fig. 3 is a sectional plan view of a modification; Fig. 4 is a side of the same showing it applied 40 to a mold; Fig. 5 is a sectional plan view of another modification; Fig. 6 is a side view of the same showing it applied to a mold; and Fig. 7 is a side view of another modification.

45 Referring to Figs. 1 and 2 of the drawings, A is any standard ingot mold of any size, shape or dimensions whatsoever with suitable lugs  $\alpha$  to which may be fastened chains, rods or other suitable means for moving the ingot mold A by means of a 50 crane, derrick or other suitable device, either before or after the feeder has been placed thereon.

B, represents the feeder which is of furnace sand, fire clay or other refractory ma-

terial and shaped to conform to the size of 55 any standard ingot, the outer diameter of the feeder being substantially the same as the inner diameter of the mold A.

Surrounding the feeder B is a solid continuous metal band C which fits sufficiently 60 loose to admit of its being moved freely upward or downward and is held in any desired position thereon by wedges D inserted between the feeder B and the band C.

It will be seen that the band C can be 65 readily adjusted on the feeder and rests loosely on the top of the mold, and firmly supports the feeder thereon.

In Figs. 3 and 4, the feeder B is surrounded by a metal band E formed of sections  $e$ ,  $e^2$ ,  $e^3$  and  $e^4$  hinged together as shown. The sections  $e$  and  $e^4$  are provided with apertured lugs  $e^5$  and  $e^6$  through which a screw  $e^7$  passes and by means of which the band is clamped upon the feeder. 75

In Figs. 5 and 6 the band F is formed of two sections  $f$ ,  $f^2$  hinged together and their free ends extended to form lugs  $f^3$  and  $f^4$  upon which fit a ring  $f^5$  and by means of which the band F is clamped upon the 80 feeder. Any other fastening means may be employed in place of the ring.

In Fig. 7 a band in the form of a chain G provided with a hook or other fastening is employed. 85

In the use of any of the above described means, it will be seen that the feeder may be inserted into the ingot mold A to any degree whatsoever, thus providing a feeder that may be used in casting ingots of greater 90 or lesser length with the same mold.

From the foregoing description taken in connection with the drawings, the method of casting ingots by the use of our adjustable feeder is as follows: Any of the various devices shown in the several figures may be used, but we prefer that shown in Figs. 1 and 2 and will describe the process of casting ingots with reference to said figures, the method being substantially the same in each 100 case.

The band C is placed in any desired position about the feeder and securely fastened by the insertion of wedges D between the outer surface of the feeder and the inner 105 surface of the band C. The feeder B with band C affixed is then placed on top of an ingot mold the lower surface of the band C

resting loosely upon top of the ingot mold A, the lower portion of the feeder projecting down into the bore of the ingot mold A, with the upper portion projecting out and above the mold.

5 While in this position, molten metal is poured into the ingot mold through the feeder which is heated to a high degree. As the molten metal comes in contact with the 10 heated feeder of refractory material, the iron or steel is held in a molten state for a considerable length of time and while in this condition will flow downward and fill any pipes that may be formed by the 15 contraction of the metal cooling below, so that a solid ingot free from pipes is produced.

We claim:

1. A feeder for ingot molds, comprising a tubular body of refractory material, and a member surrounding the feeder and adjustably secured on the feeder.

2. A feeder for ingot molds, comprising a tubular body of refractory material, a band surrounding the feeder and means for adjustably securing the band on the feeder. 25

3. A feeder for ingot molds, comprising a tubular body formed of refractory material, a band surrounding the feeder, and wedges between the band and feeder for securing it in position.

ERNEST J. TURNER.  
BLOOMFIELD H. HOWARD.